

## UNITED STATES PATENT OFFICE

2,148,331

METHOD AND COMPOSITION FOR COATING  
IRON AND STEEL ARTICLESMark Weisberg and Louis Corman, Providence,  
R. I., assignors to Alrose Chemical Company, a  
corporation of Rhode IslandNo Drawing. Application February 25, 1937,  
Serial No. 127,808

5 Claims. (Cl. 148—6.5)

This application is in part a continuation of our copending application of the same title, Serial No. 926 filed January 8th, 1935. By this reference thereto, the entire disclosure thereof is hereby incorporated herein.

This invention relates to methods and compositions for surface treating iron and steel articles with an aqueous solution containing an alkali and an oxidizing agent, for coloring or 10 coating the articles by chemical action on the surface thereof, and has for its principal objects the development of a very simple and economical aqueous solution for coating or coloring ferrous metals chemically, and a definite 15 method of control of the solution during plant operation. This invention has for other objects to avoid a large number of the following disadvantages which have rendered prior expedients along this line unsatisfactory:

20 The prior coatings have been defective in durability or appearance, being non-adherent or subject to chipping, cracking, scaling, peeling or powdering off, or unable to withstand stamping, shaping or rolling operations, or non-rust resisting, or the coating has been dull or lacking 25 beauty and depth, or not permanent, or subject to discoloring with time.

The prior processes have been expensive in 30 the cost to color a unit area, requiring costly equipment or electric set-up and power, or difficult or complicated, requiring more than one operation to complete the work such as spraying, baking, plating or hand sponging or requiring expert and skilled labor, or being incapable of 35 coloring large quantities in baskets, or yielding non-uniform results or altering dimensions or affecting hardness and elasticity of articles particularly special steels being treated.

The baths employed heretofore have required 40 expensive chemicals or high temperatures or molten salts or inflammable materials, or have been difficult to prepare or may decompose on standing idle, or have short life in operation, or leave a scum or tacky or greasy surface on 45 the article or attack the surface such as by etching the polish, or deposit oxides of metals electronegative to iron thus decreasing rust resistance, or generate excessive carbonaceous material which interferes with operation, or the bath will not work on common grades of iron 50 or steel.

Of all these disadvantages of the prior expedients along this line, perhaps the greatest or most difficult to master is that the solution ceases to function properly after a comparatively small

number of articles of ferrous metals have been coated or colored, even before the oxygen or color supplying content of the bath has been exhausted. This we have found to be due to the presence of some forms or compounds of iron 5 resulting from previous operation. Such forms or compounds are frequently formed when plain water is added to replace evaporation losses, and they are generally colloidal in nature.

It is therefore a particular object of the present invention to avoid the formation of such undesirable forms or compounds of iron resulting from previous operation, so as to prevent them from interfering with the further operation.

We attain long life for our coloring bath by 15 application of one or more of the following conditions:

(1) Control of the original composition of the solution or bath, including the optional use of inert water soluble and alkali soluble chemicals 20 in place of a considerable proportion of the alkali.

(2) Control of the temperature of operation, including the optional use of special ranges for different color effects.

(3) Addition of make up water to replace 25 evaporation losses in the form of a relatively dilute aqueous solution of alkali or oxidizing agent, or both.

With regard to the alkali to be used according to the present invention, we have found that 30 we can use any water soluble, non-volatile alkali or combination of alkalies, such as, for example, sodium hydroxide, potassium hydroxide, lithium hydroxide, sodium carbonate, potassium carbonate, sodium borate or sodium phosphate. These 35 examples are given in an illustrative and not in a limiting sense.

With regard to the oxidizing agent for our purposes we have found that we can use any material which will form an oxidizing radical 40 or substance on the bath, such as for example, a chlorate, nitrate, nitrite, oxide, nitrophenol, chromate, nitroprusside of any metal or element, but preferably the alkali metals, although the examples are given in an illustrative and not 45 in a limiting sense.

The revivifying, activating or regenerating agents which we have found to be suitable for our purpose are for example a cyanide, tartrate, bitartrate or tannate, or any other substance 50 capable of forming complex ions with that type of iron compounds shown to act as poisons or interfere with the coloring or coating action in the coloring bath, and hence the examples are given in an illustrative and not in a limiting 55

sense. These materials are activating agents or regenerating agents in the corrective sense, in that they are not necessarily oxygen bearing or color supplying substances, but instead revivify the solution by rendering active the substances already in the bath, but which have become inactive due to the presence of the undesirable form or compound of the iron which has come into the solution from the articles previously treated.

The temperature may vary from 105 to 180 degrees C. and can be attained, if necessary, by adding to the treating solution water and alkali soluble salts such as, for example, sodium chloride, sodium sulphate, potassium chloride, etc., which are generally chemically inert insofar as the coloring action is concerned.

The following is an example indicating the composition of our bath:

20 Alkali 0.3 to 8 lbs., preferably 3 lbs.  
Oxidizing agent 0.004 lb. to 10 lbs., preferably 1 lb.  
Water 4 lbs.

25 In operation this bath may be kept at a temperature range of from 105 to 180 degrees C. In case a low concentration of alkali or oxidizing agent be used it may be necessary to dissolve an inert soluble salt in the bath such as sodium chloride, potassium chloride, etc. in order to attain sufficient temperature to permit the bath to function. The concentration of this inert salt may vary from 0 to 60% of the total weight of the bath. The iron or steel articles are immersed 30 in the bath for a period of five seconds to thirty minutes, depending on the depth of coating desired, and the character of the iron or steel being treated. Activating salts may or may not be necessary to obtain satisfactory results from a 35 newly prepared bath. This depends on the result of a simple control test made by immersing a prepared steel test piece in the bath under definite conditions for a definite brief time interval.

40 45 After coating a definite amount of metal it is sometimes desirable to add a small amount of activating salts, for example, about 0.5% addition by weight of the bath, to enable the bath to continue to function satisfactorily for the coating. This addition permits a further definite amount of metal to be coated, after which a further addition of either activating salts or make up materials must be added. This process can be continued practically indefinitely, thus permitting continuous operation of the bath. There are definite limits to the amount of activating salts which can be added to the bath at any one time in order for the same to function properly.

50 55 60 The composition of the bath can be varied over a broad range and still yield satisfactory coatings. For example, the concentrations of the various components of the bath, except the activating salts, can be varied widely. Also, the permissible working temperature range is broad.

While we have emphasized above the operation employing revivifying agents, we have discovered that we can also accomplish our objects without using these additional materials.

65 70 75 It has been observed many times during our early experiments with the bath consisting of alkali, water, and nitrite, that just after replacing the water lost by evaporation during operation, the bath often though not always lost its coloring powers. To restore the coloring powers,

it was necessary to either raise the operating temperature or to add a regenerating agent. On careful investigation of this phenomenon taking place when water is added to this type of bath, it was learned that the water added reacts with the insoluble iron salts present (which were formed during previous coloring action of the bath on iron and steel articles) to form an apparently colloidal type of iron compound. To this latter compound or perhaps its reaction with the normal constituents of the bath we attribute the cause of the bath to become poisoned and stop its coloring action. The formation of this colloidal iron compound was shown by the following experiment:

A bath consisting of caustic soda, sodium nitrite, and water was operated without resort to regenerating agents. After coloring a large amount of steel articles it was decided to filter the solution through asbestos in order to free it from a heavy insoluble green sludge consisting of the iron salts formed during coloring operations. Although the filtrate was perfectly clear and practically colorless, the washings of the green iron salt sludge, obtained by pouring cold water over the filter funnel containing the sludge, were a rich red brown color. These washings on standing a few minutes yielded a flocculant red brown precipitate suspended in a colorless solution, very similar to the characteristic red brown precipitate often observed when a colloidal solution of ferric hydroxide breaks up into like constituents.

As a result of these observations a series of tests were made with a bath composed of an alkali, water, and nitrite. This bath was operated without using regenerating agents, and the losses due to drag-out of bath by the work and to evaporation were replaced from time to time by a weak solution of alkali plus nitrite. Using this manner of replacing bath losses, it was possible to obtain perfectly satisfactory coloring results, and a long life from the bath. If plain water were used to replace bath losses in above tests, the solution would have a very short life. This fact has been proven innumerable times in both laboratory experiments and in plant scale operations, while before this particular discovery we had found it necessary to add a regenerating agent from time to time to prolong the life of the bath.

The following table gives the data which was taken in experiments supporting the above statements. No regenerating agent was used in these experiments, and bath losses were replaced by a 10% solution of alkali plus nitrite.

| NaOH         | NaNO <sub>2</sub> | H <sub>2</sub> O | Operating temperature | Coloring time (min.) | Square feet of steel colored | Quality of color obtained |
|--------------|-------------------|------------------|-----------------------|----------------------|------------------------------|---------------------------|
| Grams<br>210 | Grams<br>70       | Grams<br>240     | *C.<br>(140-155)      | 5                    | 10                           | Good.                     |
| 250          | (10-30)           | 250              | (131-146)             | 5                    | 15                           | Good.                     |
| 255          | 10                | 300              | (133-144)             | 5                    | 26                           | Good.                     |
| 190          | 10                | 300              | (126-146)             | 5                    | 73 $\frac{1}{2}$             | Good.                     |

The amounts given in the column of square feet of steel colored represent amounts colored in size of bath given and are not the maximum obtainable. This feature is given so as to show the life of the bath is long. The above data is not to be construed as meaning we limit the operating conditions of the bath to those indicated. There is an appreciably wide range of practically all the factors involved.

Not only do we recognize the fact that the

- addition of plain water to this type of bath is harmful to its coloring action, but also we appreciate the fact that in entering articles to be colored into the bath, the former should not have plain water on them but preferably should be dipped in a dilute solution of caustic soda, or caustic soda plus nitrite, immediately before entering the coloring bath.

The following is a typical procedure for operating this type of bath without use of regenerating agents. Note that this procedure is given only as an example of one that has proven satisfactory and that modifications of same will yield equally good results:

- 15 Cleanse the articles in a hot alkaline cleaner, rinse in cold water, dip in an acid pickle, rinse in cold water, dip in a cold or hot 10% solution of caustic soda or a cold or hot solution containing 100 grams per liter of coloring salts (alkali plus oxidizing agent), the ratio of alkali to oxidizing agent being the same as in the coloring bath. Now, without rinsing, enter into the coloring bath at the proper operating temperature which may range from 120 to 165° C. for approximately five minutes. Remove from bath, rinse, and dry. Articles can often times be colored satisfactorily even when entered into bath without any preliminary treatment.

Thus we have made an improvement in the operation of a ferrous metal coloring bath such that regular and continuous coloring operation can be attained without the use of regenerating agents, the bath being operated substantially as above described, and resulting in a prolonged life of same.

We have also discovered the detrimental action of plain water added to a used coloring bath composed of alkali, oxidizing agent and water, and the remedy for same, namely addition of a relatively dilute solution of alkali, or alkali plus oxidizing agent to the bath in place of water.

restrict ourselves to the above listed inert water soluble chemicals nor to the amounts used as experience has shown that a wide list of these can be used with equally satisfactory results.

By increasing the concentration of chemicals in the bath and increasing the operating temperature, an interesting and valuable new coating on iron and steel is obtained. This coating is an olive green etching on the surface of the metal. It is very adherent and will absorb unusually large amounts of oil, lacquer, paint, or varnish, due to the etched nature of the coating. This type of surface results in greater protection of the steel from rusting elements for it acts as an ideal and strong bond between the metal and any lacquer, paint, or varnish put over it. Also, as it is capable of absorbing more oil due to the etched nature of the coating, a better rust protection is afforded when the colored article is oiled.

The following is an example showing the conditions required to obtain this olive green coating on steel or iron:

| NaOH      | NaNO <sub>2</sub> | H <sub>2</sub> O | Operating temperature | Coloring time | Color        |
|-----------|-------------------|------------------|-----------------------|---------------|--------------|
| Grams 750 | Grams 250         | Grams 600        | °C. 156-225           | Min. 5        | Olive green. |

25

30

In general we may say that to get the olive green coating, a high concentration of chemicals in solution is necessary, but the operating temperature and coloring time may vary over a very wide range.

Our work to determine the effect of varying concentrations of oxidizing agent shows that even lower concentrations can be used and still obtain coloring action from the bath. The following data was taken from our experiments along these lines:

35

40

45

50

We claim:

1. Method of surface treating ferrous metal articles, which comprises subjecting them to surface contact with a relatively concentrated aqueous solution containing an alkali and an oxidizing agent and having a specific gravity within the range of 1.30 to 1.60 measured at 120° C., while maintaining said treating solution at a temperature of from 105° C. to 180° C., whereby chemical action takes place on the surface of said articles, and avoiding inhibiting action of products resulting from such operation and attendant upon the addition of plain water to said concentrated solution, by adding to said treating solution to make up water losses due to evaporation, a relatively dilute aqueous solution of the order of 10% of at least one of the substances of the group named above as constituents of said relatively concentrated solution.

55

60

65

70

75

| Test No. | NaOH      | NaNO <sub>2</sub> | H <sub>2</sub> O | Operating temperature | Coloring time | NaCN    | Color on steel |
|----------|-----------|-------------------|------------------|-----------------------|---------------|---------|----------------|
| 1        | Grams 250 | Grams 0.5         | Grams 300        | °C. 140               | Min. 5        | Grams 0 | Gray etch.     |
| 2        | 250       | 2                 | 300              | 140                   | 5             | 0       | Gray.          |
| 3        | 250       | 5                 | 300              | 140                   | 5             | 0       | Black.         |
| 4        | 250       | 80                | 300              | 143                   | 5             | 0       | Do.            |
| 5        | 140       | 500               | 240              | 155                   | 5             | 0       | Do.            |
| 6        | 140       | 500               | 240              | 155                   | ½             | 5       | Rich blue.     |

We have also found it to be possible to replace a considerable proportion of the alkali in the type of bath outlined hereinbefore by inert water soluble chemicals without harming the coloring powers of the bath. The following data was taken during experiments along these lines:

| Inert water soluble chemicals                                                 | NaOH      | NaNO <sub>2</sub> | H <sub>2</sub> O | Operating temperature | Coloring time | Quality of color |
|-------------------------------------------------------------------------------|-----------|-------------------|------------------|-----------------------|---------------|------------------|
| Potassium ferricyanide 65(K <sub>4</sub> FeC <sub>6</sub> N <sub>6</sub> )... | Grams 210 | Grams 5           | Grams 240        | °C. 138               | Min. 5        | Good.            |
| Sodium chloride 70 80NaCl.....                                                | 50        | 25                | 160              | 118                   | 10            | Good.            |

For economical reasons or otherwise it may be advisable to replace part of the alkali with an inert chemical and for these reasons we made the above experiments and disclosures. We do not

2. Method of surface treating ferrous metal articles, which comprises subjecting them to surface contact with a relatively concentrated aque-

78

ous solution containing an alkali and an oxidizing agent having a specific gravity within the range of 1.30 to 1.60 measured at 120° C. while maintaining said solution at a temperature of 5 from 105° to 180° C., whereby chemical action takes place on the surface of said articles, and avoiding inhibiting action of products resulting from such operation and attendant upon the addition of plain water, by adding to said solution 10 to make up water losses due to evaporation, a relatively dilute aqueous solution of the order of 10% of at least one substance of the group consisting of alkalis, oxidizing agents, and activating agents which chemically convert such products 15 into substances harmless to the treating powers of the relatively concentrated solution.

3. Method of surface treating ferrous metal articles, which comprises subjecting them to surface contact with a relatively concentrated aqueous solution containing an alkali and an oxidizing agent and having a specific gravity within the range of 1.30 to 1.60 measured at 120° C., while maintaining said treating solution at a 20 temperature of from 105° C. to 180° C., whereby 25 chemical action takes place on the surface of said articles, employing in said solution to maintain said concentration within said temperature range a water and alkali soluble salt which is inert with respect to said chemical action, and avoiding 30 inhibiting action of products resulting from such operation and attendant upon the addition of plain water to said concentrated solution, by adding to said treating solution to make up water losses due to evaporation, a relatively 35 dilute solution of the order of 10% of at least one of the constituents of said relatively concentrated solution.

4. Method of surface treating ferrous metal articles, to produce an olive green etching on their surfaces, which comprises subjecting them to surface contact with an aqueous solution containing a caustic alkali and an alkali metal nitrate, the weight of alkali and oxidizing agent being in excess of the weight of water, and maintaining the temperature of said treating solution between 150° and 225° C. whereby chemical action 10 takes place on the surface of said articles, 15 simultaneously etching and coloring the same.

5. Bath for surface treating ferrous metal articles, comprising a relatively concentrated aqueous solution containing an alkali and an oxidizing agent and having a specific gravity within 15 the range of 1.30 to 1.60 measured at 120° C., and adapted to act chemically on said articles when maintained at a temperature of from 105° C. to 180° C., but which would become inefficient due 20 to inhibition of iron ions accumulating from said action if and when plain water were added thereto to make up evaporation losses, in combination with a pre-dip bath comprising a relatively dilute aqueous solution of the order of 10% of at 25 least one of the chemical constituents of the treating bath, and adapted to receive said ferrous metal articles in advance of treatment and thereby prevent drops of plain water from clinging to the articles and being carried into the treating bath, said pre-dip bath also being 30 adapted to make up evaporation losses from said treating bath and thereby avoid necessity of plain water for that purpose, and consequent inhibition of the action of the relatively concentrated treating bath.

35  
MARK WEISBERG.  
LOUIS CORMAN.